

1

2,974,048

**CORE BINDER**

Jacob W. Sietsema, Northbrook, Ill., assignor to International Minerals & Chemical Corporation, a corporation of New York

No Drawing. Filed Dec. 30, 1957, Ser. No. 705,793

4 Claims. (Cl. 106—38.5)

The present invention relates to cores for foundry purposes. More particularly, it relates to a foundry core of high baked strength, imparted by a novel binder component.

In the casting of metals, void spaces in the casting are produced by incorporating "cores" of one sort or another in the mold. Such cores, like the mold itself, are made of sand, and must include some kind of binding material to withstand the eroding action of the molten metal. Inasmuch as the cores are largely surrounded by the molten metal, the requirements for a satisfactory binder are a great deal more severe than for the external mold itself. A great deal of work has accordingly been done in the field of core binders. Numerous materials have been used for this purpose in the past, including cereal products, water glass, drying oils, resins, sulfite liquor, proteinaceous materials, molasses, clays, wood flour, gelatinized starches, dextrinized starches, and many other substances. In each case, it is usually found necessary to add one or more additional binder components in order to produce a core approaching the desired properties. Most of the prior-art binders are capable of producing adequate "green strength"—i.e., sufficient strength to permit the core to be transferred into a baking zone. The various prior-art materials vary greatly, however, in their so-called "baked strength" (i.e., their strength after being baked, which must be sufficient to withstand the impact and the stresses produced by the molten metal) and in their "hot properties" (these being the ability of the core to withstand the molten metal until solidification is well advanced, and then to give way thereafter so as to avoid imparting stresses in the casting). The present invention relates to an improved core binder component which has the property of imparting remarkably high baked strength in foundry cores, without interfering in any way with the hot properties thereof.

An object of the present invention is to produce an improved foundry core.

Another object is to provide an improved core binder component.

Another object is to provide a core binder component capable of imparting high baked strength without interfering with the hot properties of the core.

Another object is to segregate the fraction of gelatinized starch capable of imparting high baked strength to foundry cores, and to remove deleterious substances therefrom.

Other objects of the invention will be apparent from the present description and claims.

I have now found that gelatinized amylopectin is extraordinarily effective as a component of core binders to increase the baked strength of the resulting cores. For this purpose, gelatinized amylopectin is employed in a form substantially free from amylose and preferably substantially free from fats, proteins, fibers, and other substances commonly found in association therewith, and is incorporated in a foundry core in a proportion between about 0.1 and about 3% by weight, together with a pro-

2

portion of water between about 2 and about 6% by weight, based on the weight of the dry mixture. The amylopectin is preferably employed in the form of a dry powder, which is mulled or otherwise blended into a core sand in the desired proportion, optimally between about 0.5 and about 1.5% by weight. The water is preferably blended into the sand before the amylopectin. Amylopectin can also be added to other core-binder compositions, e.g., gelatinized starch, "cereal" (corn flour), or the like, to improve the baked strength thereof. The completed core mixture, when properly blended, formed into the desired shapes, and baked, yields cores having a baked tensile strength as high as 250 p.s.i. or more.

Starch appears to be composed of two types of molecules—a straight-chain fraction called "amylose," and a branched-chain fraction called "amylopectin." These two fractions are known to differ substantially in physical and chemical properties, such as solubility, enzyme digestibility, color formation with iodine, crystallinity, viscosity in aqueous dispersion, and in other respects. The separation of the two fractions in their original form does not appear to have been accomplished. In every case, it has apparently been necessary to subject the starch granules to at least a swelling treatment with water as a preliminary to separating the fractions. It has been reported that amylose can be extracted with hot water from swollen corn starch granules. The most effective separation technique, however, starts with a starch "paste"; i.e., a dispersion prepared by boiling starch with water. From such a dispersion, amylose can be selectively precipitated by addition of butanol or pentanol, leaving the amylopectin in solution (Schoch, *Cereal Chem.*, 18 (1941), 121; *J. Am. Chem. Soc.*, 64 (1942), 2957).

The amylopectin thus obtained is, of course, a gelatinized form of the original amylopectin. This is the material which I have found to be particularly effective in producing foundry cores of high baked strength without impairing the hot properties thereof. The dispersion can be used directly as an additive to a core mixture, preferably after distilling off the butanol or pentanol, and preferably after evaporating to produce an appropriate ratio of amylopectin and water as desired in the final core mixture. More conveniently, however, the amylopectin dispersion can be evaporated to dryness, suitably in a spray dryer or by use of a concentrator and a drum flaker, yielding a solid product which is readily stored, handled, and admixed with foundry sands. When the solid material is added to sand, the mixture should be blended, commingled with water in the desired proportion (preferably around 3 to 5% by weight) and again blended before being shaped and baked.

I have discovered that the effectiveness of gelatinized amylopectin is far in excess of what might be expected from the prior-art use of gelatinized starch in cores. It appears that the other constituents in gelatinized starch act not merely as diluents but as active adulterants, greatly reducing the effectiveness of the amylopectin. When such materials are removed (particularly the amylose), the purified gelatinized amylopectin produces a baked strength more than twice as great as might be expected from its behavior in the form of crude gelatinized starch.

Another remarkable property of gelatinized amylopectin lies in its ability to produce a "baked" core at ordinary temperature; i.e., when a core containing the purified material is merely allowed to stand at room temperature, it undergoes chemical and physical changes of unascertained nature which result in high "baked" strength without actual baking in the manner practiced by the prior art. It is, of course, feasible to carry out a conventional type of baking to hasten the process; but even when this is done, the temperatures and the baking times required may be substantially lower than in the

prior art to accomplish essentially the same result. The baking can satisfactorily be carried out, for example, at temperatures as low as around 300 to 400° F. for periods of as little as 5 to 15 minutes.

In an especially advantageous modification of my invention, gelatinized amylopectin is employed as a core binder in combination with an alkali-metal phosphate-modified starch, prepared as described by Neukom in U.S. Patents 2,884,412 (April 28, 1959) and 2,865,762 (December 23, 1958). In the Neukom method, dry, ungelatinized starch is impregnated with an aqueous solution of an alkali-metal orthophosphate salt having a pH between about 4 and about 7, optimally around 6, then dried to less than about 15% water content, and heated at a temperature between about 125 and about 200° C., preferably between about 150 and about 175° C., for a period of about 1 to about 15 hours, the heating time varying inversely with the temperature. A modified starch is obtained thereby, having the property of dispersing rapidly in cold water to produce dispersions having a viscosity between about 1,000 and about 5,000 cp., measured in 5% aqueous dispersion at room temperature. Such modified starches are highly useful in core binders, producing cores of good hot properties. The baked strength of such cores (and of foundry cores in general) is materially improved by including gelatinized amylopectin in the binder, suitably in a proportion between about 10 and about 75% by weight, based on the total binder.

As defined in Neukom U.S. Patent 2,884,412, the Neukom starch phosphates are substances prepared by impregnating an ungelatinized starch with at least about 1.0% by weight, calculated as phosphorus, of at least one phosphate salt of an alkali-metal in an aqueous solution of said salt having a pH between 3.0 and about 7.5, and heating the impregnated starch in the substantial absence of unabsorbed water at a temperature between about 120 and about 175° C. for a period of about 1 to about 15 hours.

For the preparation of phosphate-modified starches, the preferred phosphate salts are the sodium, potassium, and lithium orthophosphates, alone or in suitable combinations with themselves and/or with orthophosphoric acid to yield a pH of the desired level in aqueous solution. The impregnating solution may suitably be between about 1 and about 3 molar in phosphate, and should be used in a quantity equivalent to at least about 1% by weight of phosphorus, preferably between about 3 and about 5%, based on the quantity of starch to be treated. The starch and solution are slurried together in the desired proportion for 5 to 10 minutes or more, then separated. The starch is dried at a temperature below its gelatinization point, ordinarily below about 60-80° C., depending upon the particular starch, to a moisture content around 8 to 15% or somewhat lower, and is then subjected to heat treatment as described hereinabove. The baked material is a phosphate-modified starch suitable for use as a core binder, and advantageously useful in combination with gelatinized amylopectin in accordance with my invention.

The invention will be more clearly understood from the following operating examples. All of the tests described therein were carried out according to standard methods defined in the "Foundry Sand Handbook," Sixth Edition (1952), published by the American Foundrymen's Society, Chicago. All measurements are on a dry basis. In each case, the cores were prepared and tested in triplicate, and the reported results are the average of the three tests.

#### Example 1

The following test illustrates the use of gelatinized amylopectin alone as a core binder. The resulting core had excellent baked strength, but relatively low hot strength.

No. 1 steel sand having an AFS grain fineness of 65 ("AGF 65") was mulled with 5% by weight of water for 1 minute; then 1% of substantially pure, dry, gelatinized amylopectin was added, and mulling was continued for 6 minutes. The completed mixture retained 5.0% water. Standard test cores prepared therefrom had a green strength of 0.95 p.s.i. After they were baked 20 minutes at 425° F., their tensile strength at break was 265 p.s.i.

Standard cores were then prepared for measurement of the "hot strength" of the core mixture, measured in terms of the time required for a 1½" dia. x 2" cylindrical test core to collapse under a 100-lb. load at a given oven temperature. In each case, the test cores were baked 20 minutes at 425° F. The results were as follows:

| Oven Temp., °F. | Time for Collapse, min. |
|-----------------|-------------------------|
| 800             | 2.80                    |
| 1,000           | 1.60                    |
| 1,500           | 0.79                    |

25

#### Example 2

The following illustrates a mixed core binder consisting of a conventional cereal-type binder plus gelatinized amylopectin.

No. 1 steel sand, AGF 65, was mulled with 5% water for 1 minute; then 1% of corn flour and 0.25% of dry, gelatinized, substantially pure amylopectin were added, and mulling was continued for 6 minutes. The completed mixture retained 5.0% of moisture. Standard test cores prepared therefrom had a green strength of 0.85 p.s.i. When baked at 425° F. their strength was as follows:

40

| Baking Time, min. | Baked Strength, p.s.i. |
|-------------------|------------------------|
| 15                | 275                    |
| 20                | 260                    |
| 30                | 240                    |
| 40                | 220                    |

45

Hot-strength test cores, baked 20 min. at 425° F., had the following properties:

55

| Oven Temp., °F. | Time for Collapse, min. |
|-----------------|-------------------------|
| 800             | 3.30                    |
| 1,000           | 1.92                    |

60

#### Example 3

The following test illustrates the use of gelatinized amylopectin in combination with a technical-grade sodium phosphate-modified corn starch, prepared as described above, containing about 4.04% phosphorus and having a viscosity of 6310 cp. at 25° C. in 5% aqueous dispersion.

No. 1 steel sand, AGF 65, was mulled with 5% water for 1 minute; then 1% of a 50:50 mixture of the phosphate-modified starch and dry, gelatinized, substantially pure amylopectin was added, and mulling was continued for 6 minutes. The completed mixture contained 5.2% water. Standard test cores prepared therefrom had a green strength of 0.80 p.s.i. and a baked strength (20

min. at 425° F.) of 225 p.s.i. The baked cores had hot strengths as follows:

| Oven Temp., ° F. | Time for Collapse, min. |
|------------------|-------------------------|
| 800              | 3.43                    |

*Example 4*

The core mixture of Example 3 was repeated, except that it was prepared with 3.2% of water, and the completed mixture contained 3.1% of water. Standard test cores had a green strength of 1.05 p.s.i., and developed high baked strength at temperatures as low as 300° F.:

| Baking Time, min. | Baked Strength, p.s.i. |         |         |
|-------------------|------------------------|---------|---------|
|                   | 300° F.                | 400° F. | 450° F. |
| 10                |                        | 145     | 165     |
| 15                |                        | 185     | 175     |
| 20                | 195                    | 175     | 170     |
| 30                | 200                    |         |         |
| 40                | 185                    |         |         |

Even at room temperature, the green cores cured to a "baked strength" of 145 p.s.i. in 16 hours.

*Example 5*

The core mixture of Example 3 was repeated, except that the proportion of phosphate-modified starch to amylopectin was 40:60. The completed mixture contained 5.0% water. The test cores had a green strength of 1.25 p.s.i. and a baked strength (20 min. at 425° F.) of 250 p.s.i. The baked cores had the following hot properties:

| Oven Temp., ° F. | Time for Collapse, min. |
|------------------|-------------------------|
| 800              | 6.08                    |
| 1,000            | 2.15                    |
| 1,500            | 0.94                    |

The specific details of the foregoing examples and of the present description are submitted only for the purpose of illustrating and clarifying the invention, and with no intent to limit the invention thereto. Numerous modifications and equivalents of the invention will be 50

apparent from the foregoing description to those skilled in the art.

In accordance with the foregoing description, I claim as my invention:

- 5 1. In a method for the production of a foundry core from a mixture of sand, water, and binder, the improvement which comprises employing as said binder a starch fraction consisting of gelatinized amylopectin in a proportion sufficient to produce a core of improved baked 10 strength.
2. In a method for the production of a foundry core from a mixture of sand, water, and binder, the improvement which comprises incorporating into said mixture a starch fraction consisting of gelatinized amylopectin in 15 a proportion sufficient to produce a core of improved baked strength.

3. The method of claim 2 wherein said binder includes a starch phosphate prepared by impregnating an ungelatinized starch with at least about 1.0 percent by weight, 20 calculated as phosphorus, of at least one phosphate salt of an alkali metal in an aqueous solution of said salt having a pH between 3.0 and about 7.5, and heating the impregnated starch in the substantial absence of unabsorbed water at a temperature between about 120 25 and about 175° C. for a period of about 1 to about 15 hours, the length of the heating period varying inversely with the temperature.

4. In a method for the production of a foundry core from a mixture of sand, water, and cereal binder, the 30 improvement which comprises incorporating into said mixture as an added binder a starch fraction consisting of gelatinized amylopectin, the quantity of said starch fraction being sufficient to produce a total proportion of gelatinized amylopectin between about 10 and about 35 75% by weight, based on the total binder, whereby a core of improved baked strength is obtained.

**References Cited in the file of this patent**

**UNITED STATES PATENTS**

- 40 1,938,574 Bauer ----- Dec. 12, 1933  
 1,974,915 Giesecke ----- Sept. 25, 1934  
 2,779,693 Pacsu et al. ----- Jan. 29, 1957  
 2,884,412 Neukom ----- Apr. 28, 1959

**FOREIGN PATENTS**

- 543,202 Great Britain ----- Feb. 13, 1942

**OTHER REFERENCES**

Foundry, February 1950, page 177.